

## UNITED STATES PATENT OFFICE

ADRIAN P. ROUX, OF ORISKANY, NEW YORK, ASSIGNOR TO GENERAL CABLE CORPORATION, OF NEW YORK, N. Y., A CORPORATION OF NEW JERSEY

## METALLIC COMPOSITION AND METHOD OF MAKING THE SAME

No Drawing.

Application filed December 3, 1929. Serial No. 411,390.

This invention relates to metallic compositions in the nature of and similar to alloys and has for an object the provision of a new and improved composition of such characteristics as to render it suitable for a wide variety of uses in the industrial arts under many circumstances where extremely hard and tough materials are required. This composition has been developed with particular reference to the requirements of a wire-drawing die and although other uses will at once be apparent to those skilled in the art, nevertheless, the invention will be described with reference to its production and use as a wire-drawing die. It will, of course, be understood that the invention is not limited to the production of die material, and that the use of the material is not limited to the art of wire-drawing.

For a considerable period of time much work and experimentation have been done in an effort to develop materials suitable for dies and tools such as would not require tempering or hardening but would naturally be sufficiently hard, tough and otherwise suited to the exacting work to be performed. In this experimentation carbides of tungsten have proved most satisfactory and great progress in the art has been made along these lines. But no tungsten carbide heretofore made has been found suitable for tools or dies unless it contained a stronger metal admixed therewith. It has been too weak and brittle for tools and too brittle and rough for dies.

In order to utilize tungsten carbide for tools and dies it has been found necessary to form a composition of the same by the inclusion of one or more additional metals. Usually cobalt or a kindred metal has been used. This has been found to produce a considerably tougher and stronger substance than a simple tungsten carbide alone.

Dies made of a composition of tungsten, carbon and cobalt in the proper proportions and by suitable processes have given very encouraging results. But the metal which is added to tungsten and carbon to form a toughening matrix for the harder particles of tungsten carbide, is softer than

tungsten carbide and appears to wear away leaving minute pits in the working surface of the die resulting in breakage of the die or scratching of the wire.

According to the present invention a composition which is highly suitable for wire drawing dies is produced solely from tungsten and carbon without the addition of any further material. This alloy will be called a blended composition in contradistinction of a composition produced by the direct combination of the same materials which latter will be referred to as a simple or straight composition. Throughout this specification and claims the term "simple tungsten carbide" will be used to refer to a composition of tungsten and carbon which is formed by the primary or initial heat-produced combination of tungsten and carbon, whether the composition contains some or all of the chemical combinations of WC,  $W_2C$  etc. While no simple or straight composition of tungsten and carbon has proved at all satisfactory, I have discovered that by preparing a plurality of simple compositions of tungsten and carbon and blending them, that a very superior material is produced. This is noteworthy, because not only are the simple compositions which produce the blended material unsatisfactory alone, but a simple composition having the proportion of parts calculated from the blended material is markedly inferior if not wholly unsatisfactory.

A composition which has given highly satisfactory results contained the following ingredients:

|                                                        | Parts |
|--------------------------------------------------------|-------|
| Tungsten and carbon having $\frac{1}{2}$ to 1% carbon  | 1 90  |
| Tungsten and carbon having $3\frac{1}{2}$ to 4% carbon | 1     |
| Tungsten and carbon having $5\frac{1}{2}$ to 6% carbon | 2     |
| Tungsten and carbon having $7\frac{1}{2}$ to 8% carbon | 3 95  |

The aggregate calculated percentage of carbon is 5 5/14% to 5 6/7%. The proportions and percentages, of course, may be varied within reasonable limits. 100

- No theory can as yet be advanced regarding the state of the ingredients in the final product except that some of the material appears to form a matrix for other portions 5 of the material which have undergone further crystallization. It is difficult, in fact, to determine the state of ingredients in even a simple tungsten carbide composition. Depending upon initial proportions, such 10 a simple composition is usually found to contain the chemical compounds WC, W<sub>2</sub>C, free tungsten and free carbon. X-ray analyses of the blended compositions have been made and have shown that there is actually 15 a marked difference between the blended compositions and the straight compositions. However, sufficient tests have not yet been made to furnish a clear statement as to exactly what the controlling differences are. 20 The simple compositions may be prepared in various ways, one of which may consist in heating pure powdered tungsten mixed with pure powdered carbon in a reducing atmosphere for a number of hours at a relatively 25 low temperature say about 1100° C. (2012° F.). This operation may be effected by heating in an enclosed vitreous vessel buried in a bed of charcoal in a covered resistance furnace. 30 One illustrative method of combining the simple compositions prepared as above may be as follows: The several simple compositions in powdered form are mixed in proper proportions and placed in a carbon mold 35 closed by carbon plugs. A carbon plunger enters one end of the mold and is movable by a metal plunger so as to be capable of compressing the contents of the mold at the desired time. 40 Continuing the illustration, the filled mold is placed between water-cooled electrodes with sufficient pressure on the electrodes to establish good electrical contact with the mold; but no pressure is placed upon the 45 plunger as yet. The current is turned on to sinter the mixture in the mold. After a temperature of about 2500° F. is attained the current is turned off and simultaneously therewith sudden pressure is brought upon 50 the plunger and through it upon the sintered mixture in the mold. This appears to produce a coalescence of the sintered material. It is then left to cool between the water-cooled electrodes to form a blank. If desired the pressure may be and usually will 55 be maintained during cooling.
- Assuming that the resulting material is to be used for dies the blank thus formed is now drilled to form the die. It is observed in drilling that the material has a 60 granular appearance but may be drilled without unusual difficulty. Apparently it is not so hard to drill as a blank made with cobalt as a matrix material for the tungsten carbide. It polishes to a fine smooth sur-

face which in use wears down evenly and without pitting. This is believed to be due to the fact that the material is homogeneous, that is to say, uniformly hard, since there is no matrix of softer material to wear back 70 to produce pits between the larger particles of tungsten carbide. The pits referred to are not necessarily large, and ordinarily cannot be observed without the use of a microscope. In wire drawing work pits so small as to be observable only at about 100 diameters of magnification may harmfully affect the operation of the die. The present material does not contain pits (which may be designated as voids either before or after 80 they are partly exposed at the surface) which are large enough to cause ill effects in wire drawing work, so it may be referred to as being substantially free from voids. 85 The die thus formed proves to be sufficiently tough for wire drawing purposes. Experience has shown that the wear on the dies is very slow, for example, of dies in actual service a number have now run over 90 17 million feet of copper wire drawing from .072 to .064 in one pass and keeping the wire within 1% of gauge, without re-drilling and since the wear is not very appreciable it appears that the maximum life will be much greater. 95

Not only is the service unusually high but consistent good results have been realized, whereas dies of other compositions have given more or less uncertain results even when made as nearly under duplicated conditions as possible. It will be realized that great advantages accrue in this art in being able to consistently duplicate good results. 100

While one embodiment of the invention has been described in detail for purposes 105 of illustration, it is to be understood that various changes and modifications may be made within the scope of the appended claims.

#### What I claim is:

1. The method of making a metallic composition which comprises, making a plurality of simple tungsten carbide compositions at approximately 1100° C. or 2012° F., one having a carbon content of 1/2% to 1%, a second having a carbon content of 3 1/2% to 4%, a third having a carbon content of 5 1/2% to 6% and a fourth having a carbon content of 7 1/2% to 8%, mixing these several simple compositions and sintering in a closed carbon mold, cutting off the sintering heat at approximately 2500° F. and simultaneously applying pressure upon the sintered material in the mold and cooling the mold and contents. 115
2. The method of making a metallic composition which comprises, making a plurality of simple tungsten carbide compositions, mixing together one part having 1/2% to 1% carbon content, one part having 3 1/2% to 4% 120

carbon content, two parts having 5½% to 6% carbon content, three parts having 7½% to 8% carbon content and sintering in a closed carbon mold.

5. 3. The method of making a hard metallic composition which comprises consolidating under co-existent heat and pressure a plurality of simple separately formed carbides of tungsten varying in carbon content but all

10 falling within the range of from ½% to 8% carbon, without any other metals or binding agents, to form a coherent hard composition.

4. The method of making a hard metallic 15 composition which comprises mixing together a number of simple separately formed carbides of tungsten varying in carbon content but taken in such proportions that the calculated carbon content of the mixture is 20 between 5% and 6% without any other metal or binding agent and sintering the whole together under pressure.

5. The method of making a hard metallic 25 composition which comprises mixing together a plurality of powdered simple separately-formed carbides of tungsten of varying carbon content from ½% to 8% but taken in such proportions that the carbon content of the mixture is between 5% and 30 6%, heating the mixture to sintering temperature and exerting sudden pressure at approximately the same time that the heating is stopped.

6. As an article of manufacture, a composition body formed from a plurality of 35 diverse simple separately formed portions or bodies of tungsten and carbon without the addition of any other materials and having properties similar to a composition 40 formed, as for example, by sintering together the following pre-formed tungsten carbide portions:

|                          | Parts |
|--------------------------|-------|
| ½% to 1% carbon content  | 1     |
| 3½% to 4% carbon content | 1     |
| 5½% to 6% carbon content | 2     |
| 7½% to 8% carbon content | 3     |

and which is smooth and without pores 50 which are of a size to take up metal and become clogged during the drawing of metals such as copper, which is uniformly hard throughout any given section or surface whereby it will not become pitted in use as 55 a drawing die, and which is coherent and tough enough to be used as a drawing die, the material being markedly stronger in tensile strength than any material formed from tungsten and carbon alone at a single operation.

7. The method of forming composition bodies of tungsten and carbon alone without any other metals or binding materials which are compact, non-porous, strong and 65 smooth so as to be suitable for working tools

such as drawing dies, which comprises, separately forming a plurality of portions or bodies of tungsten and carbon each different from the other, reducing each portion to finely powdered condition, mixing the several portions together without the inclusion of any other material, and sintering the mixture and applying pressure to the metal while hot.

In testimony whereof, I have signed my name to this specification this 25th day of November, 1929.

ADRIAN P. ROUX.